

## UNITED STATES PATENT OFFICE

2,397,662

## METHOD OF PREPARING LUBRICATING OILS

Lawrence M. Henderson, Winnetka, and Weldon Grant Annable, Mundelein, Ill., assignors to The Pure Oil Company, Chicago, Ill., a corporation of Ohio

No Drawing. Application July 2, 1943,  
Serial No. 493,300

1 Claim. (Cl. 196—50)

This invention relates to a method for preparing lubricating oils of lower viscosity from lubricating oil stock of higher viscosity and is more particularly concerned with a method of preparing neutrals from cylinder stock.

It has already been proposed to prepare neutrals from bright stock by subjecting the latter to light cracking distillation. Wagner et al. Patent #2,155,745 describes a process which has been used commercially. Our invention is directed to an improved method of preparing neutrals from residual stocks.

It is common practice to add to lubricating oils pour depressants for the purpose of lowering the pour point of the oil. The pour depressant which is most widely used is that known as Paraflo. One of the difficulties experienced with oils containing pour depressants is that the product is not always pour stable, that is, some oils when subjected to temperature variations from —20° F. or lower to about 65° F. congeal at temperatures considerably above the A. S. T. M. pour point of the oil. Our invention overcomes the difficulty which is sometimes encountered with oils as heretofore made and makes possible the preparation of neutrals from cylinder stock which neutrals give pour stable blended oils when pour depressants are added thereto.

An object of our invention is to prepare less viscous lubricating oils from more viscous lubricating oil stock.

Another object of our invention is to prepare neutral lubricating oil stock from cylinder stock.

Another object of our invention is to prepare neutral oils from cylinder stock, which neutrals are pour stable when small amounts of pour depressants, such as Paraflo, are added thereto.

A still further object of our invention is to provide a method for producing a high yield of neutral oil from petroleum.

Other objects of our invention will become manifest from the following description.

In accordance with our invention, cylinder stock is subjected to a light cracking distillation in a batch semi-continuous or continuous still. As cylinder stocks suitable for our invention we may use stocks obtained from Pennsylvania grade oils or from Mid-Continent oils. The light cracking distillation of cylinder stock is carried out at atmospheric or sub-atmospheric pressure and temperatures within the range of approximately 650 to 800° F. in the manner set forth in the aforesaid Wagner et al. patent in connection with the cracking distillation of bright stock. Although the distillation may be carried out in a batch still, we preferred to carry out the cracking distillation in a semi-continuous or continuous distillation operation for the reason that higher yields of overhead or neutral stock can be obtained than in batch distillation. The reason

for this is that in batch operation it is usually necessary to leave a residuum in the still of about 10 to 12% of the charge, whereas in semi-continuous or continuous operation the residuum can be reduced to 4 to 6% or less of the total oil charged to the process. Where continuous or semi-continuous distillation is practical the oil may be heated in a pipe still and then passed to an enlarged distillation zone containing a body of oil undergoing distillation.

In the preferred method of carrying out our invention we maintain the temperature of the cylinder stock undergoing cracking distillation in the neighborhood of approximately 700° F. and inject into the cylinder stock an amount of live steam approximately equivalent to the amount of oil vapors taken overhead from the still. We have found that if the distillation of cylinder stock is properly conducted, yields of distillate in excess of 90% can be obtained. The distillation is preferably conducted at such a rate and at such temperature that the viscosity of the overhead stream is maintained at approximately 100 Saybolt at 100° F.

In the distillation of the cylinder stock it is advantageous to add a small amount of low boiling hydrocarbon, such as kerosene, to assist in the distillation.

The overhead stock from the light cracking distillation of the cylinder stock will have a high pour point due to the presence of crystalline or semi-crystalline wax in the oil. The presence of this wax interferes with conventional centrifugal or filter press dewaxing of the stock. We have discovered, however, that if a small amount of petrolatum, obtained by conventional cold centrifugal dewaxing of naphtha-cylinder stock solutions, is added to the overhead stock, the stock is readily amenable to centrifugal dewaxing. In accordance with our invention, therefore, we added to the overhead stock approximately 5 to 20% of petrolatum, preferably in the form of a naphtha solution, after which the stock is subjected to centrifugal dewaxing in the presence of naphtha in the conventional manner.

Before dilution of the stock with naphtha for centrifuging, it may be desirable to remove from the overhead stock low boiling hydrocarbons within the gasoline, kerosene and gas oil range. In the dewaxing operation, which may be carried out at a temperature of approximately —35° F. the higher melting waxes are removed and an oil having a pour point of approximately 25° F. may be obtained. This material is preferably blended with the proper proportions of bright stock and neutrals to the desired viscosity and will be found to respond to Paraflo and other pour depressants, so that the pour of the blend can be reduced to approximately —30° F. by ad-

dition of 1% of Paraflow, and the pour point of the oil will remain stable.

If desired, the overhead stock made by the light cracking distillation after addition of the petroleum and centrifugal dewaxing may be blended with pressed distillate and subjected to distillation to reduce to desired viscosity in the manner set forth in Wagner et al. Patent #2,155,745.

As an example of the invention, cylinder stock from a Pennsylvania oil having the following characteristics:

|                             |      |
|-----------------------------|------|
| A. P. I. gravity            | 25.0 |
| Pour, °F                    | 90   |
| Saybolt viscosity at 210° F | 143  |
| Flash, °F                   | 545  |
| Fire, °F                    | 600  |

was subjected to a light cracking distillation in a semicontinuous operation at a temperature of 690 to 710° F. Superheated steam at a temperature of 550° F. was injected into the cylinder stock in a ratio of one part by weight of steam to one part by weight of oil vapor taken overhead. The cylinder stock was mixed with kerosene prior to distillation. The following table gives the quantity of materials charged and the yield obtained based on the cylinder stock charged:

Table I

|                        | Cubic centi-meters | Percent based on cylinder stock |
|------------------------|--------------------|---------------------------------|
| Cylinder stock charged | 42,177             | 100                             |
| Kerosene charged       | 1,000              | —                               |
| Kerosene recovered     | 1,000              | —                               |
| Cracked overhead       | 38,494             | 91.2                            |
| Still bottoms          | 3,383              | 8.0                             |
| Loss                   | 300                | 0.8                             |

The cracked overhead was divided and each of two 5-gallon samples was subjected to conventional naphtha cold centrifugal dewaxing in a super centrifuge. To one sample 15% of petrolatum was added prior to centrifuging. The characteristics of the samples before and after addition of petrolatum were as follows:

Table II

|                             | Sample before addition of petrolatum | Sample after addition of petrolatum |
|-----------------------------|--------------------------------------|-------------------------------------|
| A. P. I. gravity            | 32.7                                 | 33.9                                |
| Saybolt viscosity at 100° F | 101                                  | 167                                 |
| Pour, °F                    | +90                                  | +65                                 |
| Flash, °F                   | 120                                  | 125                                 |
| Fire, °F                    | 175                                  | 135                                 |

Before dewaxing, both samples were subjected to distillation with 300° F. steam in order to remove light ends which might interfere with the blending and dewaxing with naphtha. The characteristics of the two samples after removal of the light ends were as follows:

Table III

|                           | Sample without petrolatum | Sample with petrolatum |
|---------------------------|---------------------------|------------------------|
| A. P. I. gravity          | 29.3                      | 29.9                   |
| Pour, °F                  | +90                       | +05                    |
| Flash, °F                 | 390                       | 390                    |
| Fire, °F                  | 465                       | 440                    |
| Percent residue remaining | 79.1                      | 80.4                   |

Each of the stocks, after removal of the light ends, was blended with three parts by volume of

62.1 A. P. I. gravity naphtha and chilled non-shock from 100° F. to -35° F. The chilled solutions were then centrifuged and the resulting oil and wax cake examined after separating the naphtha from each. The following table gives the results obtained from the examination of the products of the dewaxing operation:

Table IV

|                                                       | Sample without petrolatum | Sample with petrolatum |
|-------------------------------------------------------|---------------------------|------------------------|
| Oil-naphtha solution, vol. percent of charge          | 87                        | 88.4                   |
| Vol. percent oil in oil-naphtha solution              | 22.4                      | 21.6                   |
| Vol. percent 62.1 gr. naphtha in oil-naphtha solution | 77.6                      | 78.4                   |
| Vol. percent yield of oil based on charge             | 78.7                      | 79.6                   |
| Characteristics of dewaxed oil:                       |                           |                        |
| A. P. I. gravity                                      | 28.3                      | 28.7                   |
| Pour, °F                                              | 25                        | 25                     |
| Flash, °F                                             | 390                       | 390                    |
| Fire, °F                                              | 465                       | 445                    |
| Color                                                 | (1)                       | (1)                    |
| Wax cake, vol. percent of charge                      | 13                        | 11.6                   |
| Vol. percent wax in cake                              | 40.6                      | 42.0                   |
| Vol. percent of 62.1 gr. naphtha in wax cake          | 59.4                      | 58.0                   |
| Vol. percent yield of wax based on charge             | 13                        | 11.6                   |
| Characteristics of wax:                               |                           |                        |
| A. P. I. gravity                                      | 31.9                      | 34.2                   |
| M. P., °F                                             | 120                       | 128                    |
| Appearance                                            | (2)                       | (3)                    |

30 1 Dark green.

2 Semi-crystalline.

3 Amorphous.

35 The wax obtained from the operation on the overhead stock to which petrolatum stock had not been added was partly crystalline and could not be continuously discharged from a super centrifuge, whereas the wax obtained from the sample to which the petrolatum stock had been added was amorphous and the stock could be satisfactorily dewaxed in a super-centrifuge. Moreover, in spite of the addition of the 15% of petrolatum to one sample, the yield of wax was less than that obtained from the sample to which petrolatum stock had not been added, thereby indicating that in the latter operation a good separation of oil and wax had not been obtained. Moreover, the yield of dewaxed lubricating oil from the blend containing petrolatum was increased by approximately the percent of petrolatum added. This is a decided advantage since petrolatum is worth considerably less than the lubricating oil.

40 45 50 55 A 10W S. A. E. lubricating oil was made by blending together the dewaxed oil to which petrolatum has been added before dewaxing, Pennsylvania bright stock and Pennsylvania neutrals in the following proportions:

|                       | Parts by volume |
|-----------------------|-----------------|
| Dewaxed cracked stock | 77              |
| Bright stock          | 10              |
| Neutrals              | 13              |

60 The characteristics of the bright stock and neutrals used in the blend were as follows:

Table V

|                             | Bright stock | Neutrals |
|-----------------------------|--------------|----------|
| A. P. I. gravity            | 26.9         | 35.0     |
| Pour, °F                    | +15          | +30      |
| Saybolt viscosity at 100° F | 150          | 65       |
| Saybolt viscosity at 210° F |              |          |

65 70 To the blend was added 1% by volume of Paraflow and the resulting product was tested for pour point and for slow and rapid cycle pour stability.

Slow cycle pour stability is determined by fill-

ing to the mark pour jars used in making pour point determinations under A. S. T. M. designation (D-97-39) with oil samples at room temperature. The samples are placed in a 1-gallon capacity Thermos jug. In one sample is inserted a short thermometer through the cork stopper in the pour jar so that the top of the mercury bulb is  $\frac{1}{8}$  inch below the surface of the oil in the jar. The other samples in the jug are stoppered only. The pour jars should be placed in the jug in a single row around the inside wall. The jug is then tightly covered and placed in a refrigerator maintained at  $-40^{\circ}$  F. for a sufficiently long time (preferably overnight) to cool the oil samples down to  $-25^{\circ}$  F.

After the samples have cooled to  $-25^{\circ}$  F. or lower, the jug is removed from the refrigerator, the samples are removed from the jug and permitted to warm up to  $65^{\circ}$  F. (plus or minus  $5^{\circ}$  F.) without applying heat. The Thermos jug should be covered as soon as the oil samples are removed so that the inside of the jug remains reasonably cool. It will take the oil samples approximately 1 hour to warm up from  $-25^{\circ}$  F. to  $+65^{\circ}$  F. by standing in a room at a temperature of approximately  $75^{\circ}$  F. The samples should be preferably separated during the warming-up period and upon attaining a temperature of approximately  $65^{\circ}$  F. should be clear and not hazy.

As soon as all the samples have warmed up to approximately  $65^{\circ}$  F. they are returned to the Thermos jug; the Thermos jug is covered and allowed to remain in the laboratory atmosphere for 2 hours. The temperature of the oil samples is dropped from approximately  $65^{\circ}$  F. to approximately  $40^{\circ}$  F. in the two hours during which the jug is left standing in the room. Thereupon the jug is placed in a refrigerator maintained at  $-10^{\circ}$  F. and the condition of the oil is observed hourly from the time the temperature reached  $+25^{\circ}$  F. until a temperature of  $+20^{\circ}$  F. is reached. Cooling will occur at the rate of 5 to  $7^{\circ}$  F. per hour during the time the temperature of the samples dropped from  $+30$  to  $+20^{\circ}$  F. If any samples become solid before the temperature of  $+20^{\circ}$  F. is reached they are removed from the jug and the temperature recorded at which the sample became solid. When the temperature of  $+20^{\circ}$  F. is reached, the jug is removed from the refrigerator and placed in a second refrigerator maintained at  $-40^{\circ}$  F. and the temperature and condition of the oil observed hourly. Care should be exercised not to disturb the oil more than is absolutely necessary when making hourly observation.

In extremely warm weather it may be necessary to make observations every hour and a half instead of every hour in order to maintain the desired cooling rate of the samples. The test need not be taken below  $-25^{\circ}$  F. on the second cycle and oils remaining fluid down to the A. S. T. M. pour point of the sample are considered satisfactory from the standpoint of this test but such samples must still pass the rapid cycle test.

In making the rapid cycle pour stability test, the pour jars are filled to the mark with the oil samples at room temperature. Thermometers are inserted as in the A. S. T. M. pour test and a heavy cardboard gasket having an outside diameter  $1\frac{1}{2}$  inches larger than the outside diameter of the pour jars is snugly fitted on the outside of the pour jars and rests on the top of the jacket surrounding the pour jar, so that the gasket closes the space between the pour jar and the jacket.

The pour bath is cooled as rapidly as possible to  $-40^{\circ}$  F. When the oil samples reach  $-25^{\circ}$  F. they are removed from the pour bath and are permitted to warm up to  $65^{\circ}$  F. (plus or minus  $5^{\circ}$  F.) as in the slow cycle test. After the samples warm up to the  $65^{\circ}$  F. temperature they are returned to the pour bath which is now maintained at approximately  $-30^{\circ}$  F. The samples are allowed to cool down to  $+20^{\circ}$  F. and the pour bath is then rapidly cooled to  $-40$  or  $-45^{\circ}$  F. The condition of the oil samples is observed at  $-20^{\circ}$  F. for oils with a pour point of  $-25^{\circ}$  F. or lower, and at a temperature of  $10^{\circ}$  above the pour point of the oil for oils having a pour point above  $-25^{\circ}$  F. The condition of the oil is recorded as fluid or solid at the temperature of observation. Oils which remain fluid under these conditions are considered to be satisfactory as far as this test is concerned. In testing the oil to determine whether it is fluid or solid, the A. S. T. M. pour procedure is used; that is, the jar is held in a horizontal position for not more than 5 seconds.

The pour test and pour stability results on the blend are given in Table VI:

Table VI

| A. S. T. M.<br>pour | Pour stability                                                        |                                            |
|---------------------|-----------------------------------------------------------------------|--------------------------------------------|
| $-20^{\circ}$ F.    | Slow cycle:<br>Fluid at $-15^{\circ}$ F.<br>Solid at $-20^{\circ}$ F. | Rapid cycle at $-10^{\circ}$ F.;<br>Fluid. |

The pour point of the blend was satisfactory and the tests indicate that the blend had satisfactory pour stability.

It will be seen, therefore, that by subjecting cylinder stock to a light cracking distillation and then blending with a small amount of petrolatum, the resulting product can be dewaxed by conventional methods to give a product which is pour stable in the presence of small amounts of Paraflo or other pour depressants. By cracking cylinder stock instead of bright stock a higher yield of finished product can be obtained at lower cost than can be obtained by cracking bright stock, due to the fact that in our process the steps of percolation of cylinder stock through clay and cold centrifuging of the stock to remove wax are avoided. The percolation step involves unnecessary loss of desirable material.

We claim:

The method of preparing lubricating oil which comprises distilling cylinder stock from Pennsylvania oil under light cracking conditions at a temperature of approximately  $700^{\circ}$  F. at pressures not substantially above atmospheric pressures in the presence of a light hydrocarbon diluent, injecting steam into the body of cylinder stock undergoing distillation at such rate that the volume of steam is approximately equal to the volume of hydrocarbon vapors produced, condensing the vapors, continuing the distillation until approximately 91.2% by volume of the cylinder stock is distilled, adding to the distillate approximately 15% of petrolatum, removing from the mixture fractions boiling within and below the gas oil range, diluting the remainder with naphtha, chilling the solution to a temperature of approximately  $-35^{\circ}$  F., centrifuging it to remove wax and removing the naphtha from the dewaxed oil.

LAWRENCE M. HENDERSON.  
WELDON GRANT ANNABLE.